

Patented June 28, 1927.

1,633,594

# UNITED STATES PATENT OFFICE.

ELBERT C. LATHROP, OF PHILADELPHIA, PENNSYLVANIA, AND TREADWAY B. MUNROE, OF FOREST GLEN, MARYLAND, ASSIGNEES, BY DIRECT AND MESNE ASSIGNMENTS, TO DAHLBERG & COMPANY, INC., OF CHICAGO, ILLINOIS, A CORPORATION OF DELAWARE.

## RETTED BAGASSE FIBER AND PROCESS OF PRODUCING SAME.

No Drawing.

Application filed June 20, 1924. Serial No. 721,366.

This invention relates to retted bagasse fibers and process of producing the same, and has for its object to improve the fibers heretofore produced from bagasse, while at the same time preserving said fibers from deterioration, in a manner more simple and less costly than has been heretofore proposed.

With these and other objects in view, the invention consists in the novel retted bagasse fiber and in the novel steps and combinations of steps constituting the process, all as will be more fully hereinafter disclosed and particularly pointed out in the claims.

In order that the precise invention may be the more clearly understood, it is said:— In the manufacture of heat insulating and building boards or lumber from bagasse and analogous fibers, it is desirable to separate the fiber bundles more or less completely into single fibers, and this has been heretofore attempted by cooking the fibers either in water or in alkaline, or in acid solutions. After said fibers are thus cooked, they are subjected to a washing action and then to the mechanical working of the fibers in beaters called "Jordan" engines, or in "Clafin refiners," so that the fiber bundles are more or less broken up, and single fibers or smaller fiber bundles are formed from the larger bundles.

This mechanical treatment, however, is more or less costly, and furthermore it is carried out imperfectly in the machinery now employed, due to the strong cementing action of the parenchyma tissue and pith which bind the single bagasse fibers into fiber bundles. While this parenchyma tissue should be removed entirely by the cooking processes if strong chemicals are employed, yet it is well known that such cooking is difficult to control, and especially when more or less strong chemicals are employed, because in such cases it is very difficult to prevent the destruction of the strength of the fibers themselves, and further such treatment with strong chemicals is quite expensive.

According to this invention, on the other hand, it has been discovered that the desired removal of this said parenchyma tissue, which cements the fibres together in bundles,

may be brought about in such a way that but little, if any, cooking and mechanical refining is required. It thus results that when this invention is followed, a less loss of valuable fiber constituents is involved than by the now commonly practiced chemical cooking processes. Furthermore, the pulp manufactured from such retted bagasse fibers possesses certain properties not attained by the pulp that has been heretofore manufactured, as will presently appear.

In order to still further make clear the precise nature of this invention, it is also said:—Bagasse fibers as they leave the sugar cane mill contain about 50 per cent moisture and varying but small amounts of unextracted sugar, depending on the particular mill operations to which they have been subjected. It is well known that such bagasse can be immediately dried and by this means all fermentation changes can be prevented, since it is well known that micro-organisms require water in order to grow and carry on their processes of metabolism commonly called fermentation. But, again, such drying procedure is found to be too costly to render it desirable commercially, and the resulting bagasse fiber is in addition found to be harsh, and the individual fibers themselves are found to be held for the most part in the form of firm bundles due to the above-mentioned parenchyma tissue and therefore they must be subjected to cooking and refining procedures before they can be made into a satisfactory pulp.

On the other hand, if the green masses of bagasse are piled either loose or in bales, as they come from the mill with the varying water contents they possess, fermentation as is well known sets in. It therefore follows that if one simply piles a mass of bagasse as it comes from the mill, the growth of certain groups or types of bacteria, fungi or mushrooms, is favored or inhibited, depending upon the chance conditions of the particular temperature, the particular moisture content, the oxygen supply, or the hydrogen ion concentration with which the mass may have been associated. It thus results that the particular type of fermentation, and therefore of final product, is very uncertain, for each may be quite different in different masses that have been treated alike, and

also the amount of heat produced in the different masses will vary according to said chance conditions.

Of these organisms, there have been found bacteria, trichoderma, monilla, Fusarium, Aspergillus, Penicillum, Mucors, and various species of mushrooms to be present under various conditions, but in studying the effect of the organisms on bagasse fiber, both in the case of pure and in the case of mixed cultures, it has been discovered that certain of the organisms are quite selective in their attack on bagasse constituents. In particular, it has been discovered that the mushrooms are selective in their fermentation changes under controlled conditions. Certain types of mushrooms in pure cultures on bagasse, and in bales of bagasse, have been studied in the field as to their action, and it has been found that these mushrooms attack the parenchyma tissue in preference to the bagasse fiber so that this said tissue was partly or completely destroyed, leaving the bagasse fiber practically untouched.

Masses of bagasse, which have been so fermented, are of a yellowish color, and when such masses are rubbed between the hands, the individual fibers are partially or wholly separated from the fiber bundles, so that the mass seems much softer and more pliable than was the bagasse before such fermentation or retting. Studies on the diameters of fibers produced by such mushroom retting as compared with the unretted bagasse fibers which have been treated by the prior cooking and refining procedures have shown that on the average the retted fibers are of a satisfactory uniform character and quality, are of a smaller diameter and that they show a larger proportion of single fibers produced by the retting process than have been heretofore produced by the cooking and refining processes. It has also been found that a number of species of mushrooms will produce the desired retting action, such for example as *Hypholoma*, *Agaricus*, *Coprinus*, *Corticarius* or *Psilocybe*. It has been discovered that the *Psilocybe* species may be easily grown in a pure culture, and while one may carry out this invention by the use of other species, one way in which to perform this process is by the use of the said *Psilocybe* mushrooms.

*Psilocybe* and similar mushrooms are found to grow best on bagasse at a moisture content above 60 per cent and at temperatures normal to cane growing countries. The conditions of oxygen supply and hydrogen ion concentrations are also found to be important. That is, it is found that *Psilocybe* grows well at a hydrogen ion concentration (pH) of 4.0 to 5.5, and that it develops rapidly in compacted masses of bagasse such as are produced by baling in

the well known manner described in U. S. Patent No. 1,479,419, for Method of preserving bagasse fibers, etc., dated January 1, 1924, and issued to T. B. Munroe. But in this invention no alkali or other chemical is added to the bagasse previous to the baling of the same or during the process of retting said bagasse.

As is well known, the green bagasse as it leaves the mill, and when either in loose piles or in bales, at first undergoes an alcoholic and then an acetic or other acid fermentation. It has been found if water is not then supplied to the bagasse approximately 50 per cent, the bales will heat up under this fermentation and may be substantially sterilized by the heat thus generated. In order to ret the bagasse, however, by this invention, the moisture content of the bagasse in which the cultures are started should be raised above 60 per cent to preferably from 70 per cent to 80 per cent, although a higher moisture content is not objectionable.

The cane growing soils in general are found to have in them growing mushrooms, or spores of mushrooms, and therefore the cane is already inoculated with certain species of mushrooms when the bagasse is made at the mill. Especially is it found that the cane growing soils of the Southern States contain the species of mushrooms known as *Psilocybe*. It is also found that the growth of the mushroom will be favored by the conditions of moisture and temperature above noted, and in carrying out the present invention, one brings about those conditions which will induce an optimum growth of the desired species of mushroom. That is, in those cases where the cane itself is not sufficiently inoculated with mushroom fruiting bodies, or spores, one may in carrying out this invention inoculate the bagasse itself, either while it is being baled, or later, by using soil that is inoculated with the desired species of mushroom or other cultures, such for example, as *Psilocybe*. In carrying out this inoculation, one may also employ previously retted baled bagasse or he may use pure cultures of *Psilocybe*, especially grown in suitable and well known media.

It has further been found that it is not necessary to inoculate or start the growth of mushrooms in all of the bales of a pile of bagasse, or even in all parts of a mass of loose bagasse. It is found sufficient if the outer bales of a pile of bagasse are well inoculated for good growths of the *Psilocybe* are induced by the control of the moisture and temperature above mentioned. That is, the organisms will penetrate to drier bales of the pile and will grow into and through such bales, producing yellow retted bagasse fibers. This penetration is quite rapid, if the conditions of temperature and

moisture are favorable, but the high moisture content of the inner bales of the pile is not required, because during growth, the mushrooms themselves produce sufficient water by their fermenting action to wet the entrance spot or spots in adjacent bales. By controlling the moisture content of the bales, the fermentation of the bagasse and the destruction of the pith and parenchyma tissue 10 is likewise controlled; therefore by controlling the moisture present the tendency for the organism to attack the true fiber is substantially eliminated. It is further found that sterilized bagasse, after it has cooled 15 down sufficiently, is one of the most suitable forms in which to produce the retted bagasse. That is the *Psilocybe* is about the only type that will grow in such sterilized bales for the conditions for growth of other organisms 20 have been made unfavorable by the process of sterilization.

It is still further found that when piles of bagasse which have been retted are opened up, it is observed that the bales on the inside 25 of the piles appear as whitish bales on their outsides, the interior of such bales being yellow and the bales themselves being substantially dry. But the fiber of such interior bales is found to be strong and some of the 30 pith and parenchyma tissue will have been found to be destroyed, so that on mechanical rubbing, such a shredding of the fibers takes place that they will fall apart, there being present a larger proportion of single fibers 35 or small fiber bundles than have been found in bagasse not so retted.

Although it is to be understood that the invention may be carried out in other ways without departing from the spirit thereof, 40 one manner in which it may be performed is as follows:

The bagasse is baled in a compacted mass such as that described in U. S. Patent No. 1,479,419, above mentioned, with the exception that no lime or other chemical is added 45 to the bagasse as it leaves the sugar mill prior to baling. About 50 per cent of moisture remains in the bagasse after baling and the bale is so compacted that very little heat 50 escapes therefrom.

During the control of fermentation of this material, or within the course of a day to a few days, the alcoholic and lower fatty acid 55 fermentation will begin, at which time a production of carbon dioxide begins and the bales heat up. The bales are preferably then laid into piles of several hundred or thousands of bales to a pile, so that the proportion of bales exposed to the direct 60 weather is small as compared with the bales not so exposed. The bales are so placed in the piles that air channels are formed within the pile, both laterally and vertically. The 65 purpose of these air channels is to supply air currents to remove the vapors and gases

from the bales, during the pasteurization process, and to supply oxygen so as to limit the growth of certain types of organisms which are effective in producing other conditions of fermentation than those producing the pasteurizing effect. If the bales are 70 too closely packed in piles, carbonizing and scorching of the fibers is apt to take place. If disposed in small piles, or with exceedingly large air channels the heating may be 75 of too short a duration to pasteurize and sterilize the mass. During storage, under the above conditions, a substantial sterilization takes place and the moisture content of the whole bale is markedly lowered, but particularly the outside of the bales are dried out so that at touch and sight the bales appear entirely dry. If kept dry, substantially no further fermentation takes place, for the heating up and drying out process will have 80 destroyed the microorganisms which bring 85 about the effective fermentation process.

Instead of covering the bales with loose bagasse at the time of piling, the bales may be piled without any cover. In so doing, 90 the heat is more quickly removed from the interior of the pile, permitting the desired temperature conditions for retting to become favorable at an earlier period. The moisture that is condensed on the under sides 95 of the top bales, is found to supply the high moisture conditions necessary for the beginning of the germination and growth of the mushroom. In about three to six weeks, if the mushroom growth by such condensation of vapor is not sufficiently well started, 100 the outer bales should be wetted in a suitable manner, and if desirable they may be also wetted with a mixture of mushroom mycelium and micro-spores in a suitable 105 dilutent such as a media or water. The acid condition produced by fermentation in this process causes the mushrooms to start their growth and penetrate from bale to bale so that in a period of a month to several 110 months the entire mass of bagasse is substantially retted. In order to protect the bales of a pile, from secondary fermentations such as that produced by slime molds after such time as the mushroom organisms have 115 penetrated well into the pile, the top bales of the pile are broken and spread over the other bales as loose bagasse to form a layer approximately eight inches in depth, a small amount of venting being provided to carry 120 off the carbon dioxide vapors produced during the retting.

It will now be clear that this invention provides a procedure by which one may pile green bagasse from the mill either in masses 125 or in bales, allow it to go through an alcoholic fermentation, and so regulate the temperature thus generated throughout the mass as to substantially pasteurize the same without injury to the fibers. After this pasteur-

ization by heat has been accomplished, one then examines the mass to find if it still is inoculated with organisms of the mushroom type and especially of the type of 5. *Psilocybe*. If this mushroom type of fermenting organism is not present in sufficient quantities, the bagasse masses are then suitably inoculated therewith, and the bagasse left to the action of said growths. The mass 10 if too dry should be moistened in order to start the mushroom fermentation or retting action, and a moisture content above 60 per cent should be supplied and maintained.

After the retting action is once started, 15 however, the mushroom organisms will by their fermenting action supply additional moisture so that the retting action spreads rapidly throughout the mass, no matter how large it may be. These mushroom types 20 of organisms are found to attack the parenchyma tissues binding the fibers together in bundles, and they thus loosen said fibers, rendering it unnecessary to subsequently cook and mechanically beat the same to the 25 extent heretofore found necessary with un-retted fibers during pulp making processes. Further, by controlling the temperature and the moisture content, the retting action of the organisms can also be controlled and the 30 fibers recovered with their strength and flexibility unimpaired.

The retted fibers themselves are found to be of a yellow color, more pliable, and of a smaller diameter than those produced by 35 the prior cooking and refining procedures.

It will further be clear that instead of sterilizing the bagasse as above disclosed, it may be inoculated, with a number of different mushroom types of organisms and 40 retted with improved results.

It will also be clear that this invention is not limited to bagasse fibers, for analogous fiber producing materials such as bamboo, cornstalks, rice straw, and even wood, may 45 be similarly treated to advantage. For in all cases the raw fibers through this retting action are so separated from the bundles in which they are bound by nature, that it is less costly to handle them in the subsequent 50 cooking and refining procedures.

What is claimed is:—

1. The process of preparing fiber producing material for the production of pulp which consists in subjecting said material to the fermenting action of micro-organisms of the mushroom type.

2. The process of preparing fiber producing material for the production of pulp which consists in acidifying said material 60 by subjecting the same to an alcoholic and acid fermentation and then to the fermenting action of micro-organisms of the mushroom type.

3. The process of preparing fiber producing material for the subsequent production 65

of pulp which consists in subjecting said material in the presence of a predetermined water content to the fermenting action of micro-organisms of the mushroom type.

4. The process of preparing fiber producing material for the subsequent production of pulp which consists in subjecting said material in the presence of a predetermined water content and within a predetermined range of temperature to the fermenting action of micro-organisms of the mushroom type. 70 75

5. The process of preparing fiber producing material for the subsequent production of pulp which consists in subjecting said material in the presence of a predetermined water content and within a predetermined temperature range first to an alcoholic fermentation and then to the fermenting action of micro-organisms of the mushroom type. 80 85

6. The process of preparing fiber producing material for the subsequent production of pulp which consists in subjecting said material to an alcoholic fermentation; bringing said fermented material to a predetermined range of temperature and to a predetermined moisture content and subjecting the same to the fermenting action of a micro-organism of the mushroom type. 90

7. The process of preparing fiber producing material for the subsequent production of pulp which consists in subjecting said material to an alcoholic fermentation; so controlling the temperature of said material during said fermentation as to partially sterilize the same; bringing said fermented material to a predetermined range of temperature and to a predetermined moisture content and subjecting the same to the fermenting action of a micro-organism of the 100 mushroom type. 105

8. The process of preparing fiber producing material for the subsequent production of pulp which consists in subjecting said material to an alcoholic fermentation; causing 110 the heat developed by said fermentation to sterilize said material to a substantial extent; bringing said fermented material to a predetermined range of temperature and to a predetermined moisture content and subjecting the same to the fermenting action of a micro-organism of the mushroom type known as *psilocybe*. 115

9. The process of preparing fiber producing bagasse material for the production of pulp which consists in subjecting said material to the fermenting action of micro-organisms of the mushroom type. 120

10. The process of preparing fiber producing bagasse material for the subsequent production of pulp which consists in subjecting said material in the presence of a predetermined water content to the fermenting action of micro-organisms of the mushroom type. 125 130

11. The process of preparing fiber producing bagasse material for the subsequent production of pulp which consists in subjecting said material to an alcoholic fermentation; bringing said fermented material to a predetermined range of temperature and to a predetermined moisture content and subjecting the same to the fermenting action of a micro-organism of the mushroom type.

12. The process of retting bagasse fibers which consists in subjecting a mass of bagasse to an alcoholic fermentation; causing its water content to exceed 60%; and subjecting said mass to the fermenting action of a micro-organism of the mushroom type.

13. The process of retting bagasse fibers which consists in subjecting a mass of bagasse to an alcoholic fermentation; causing the heat generated to sterilize said mass to a substantial extent; causing its water content to exceed 60%; and subjecting said mass to the fermenting action of a micro-organism of the mushroom type.

14. The process of retting bagasse fibers which consists in subjecting a mass of bagasse to an alcoholic fermentation; causing its water content to exceed 60%; and subjecting said mass to the fermenting action of a micro-organism of the mushroom type known as psilocybe.

15. The process of preparing bagasse fibers for pulp making purposes; which consists in subjecting a mass of bagasse to an alcoholic fermentation; and then to a fermenta-

tion brought about by micro-organisms of the mushroom type under predetermined controlled conditions of temperature, water content and oxygen supply.

16. The process of preparing bagasse fibers for pulp making purposes, which consists in subjecting a mass of bagasse to an alcoholic fermentation; and then to a fermentation brought about by micro-organisms of the mushroom type known as psilocybe under predetermined controlled conditions of temperature, water content and oxygen supply.

17. The process of preparing bagasse fibers for pulp making purposes, which consists in subjecting a mass of bagasse to an alcoholic fermentation; substantially sterilizing said mass; and then subjecting said mass to a fermentation brought about by micro-organisms of the mushroom type known as psilocybe under predetermined controlled conditions of temperature, water content and oxygen supply.

18. The herein described new article of manufacture consisting of a mass of bagasse fibers yellow in color, pliable, of a less average diameter than those ordinarily produced by cooking and beating procedures, and produced by the retting action of micro-organisms of the mushroom type.

In testimony whereof we affix our signatures.

ELBERT C. LATHROP.  
TREADWAY B. MUNROE.